

# United States Patent [19]

ichioka

[11] 3,887,440

[45] June 3, 1975

[54] METHOD OF MANUFACTURING A  
CONTINUOUS MAGNETIC FOIL BY  
ELECTRODEPOSITION

[75] Inventor: Satoshi Ichioka, Toda, Japan

[73] Assignee: Mishima Kosan Co., Ltd.,  
Kitakyushu, Fukuoka Prefecture,  
Japan

[22] Filed: Jan. 24, 1974

[21] Appl. No.: 436,376

[52] U.S. Cl. 204/13; 204/28; 204/43 T;  
204/129.9; 204/208

[51] Int. Cl. C23b 7/04; B23p 1/00; C23b 5/68

[58] Field of Search 204/12, 13, 27, 28, 206,  
204/208, 211, 129.9

[56] References Cited

UNITED STATES PATENTS

2,433,441 12/1947 Davidoff 204/208

|           |        |                    |           |
|-----------|--------|--------------------|-----------|
| 3,639,217 | 2/1972 | Shukovsky .....    | 204/35 R  |
| 3,645,857 | 2/1972 | Fisher et al. .... | 204/28    |
| 3,647,654 | 3/1972 | Toledo et al. .... | 204/129.9 |
| 3,738,922 | 6/1973 | Toledo. ....       | 204/129.9 |

FOREIGN PATENTS OR APPLICATIONS

1,807 1/1969 Japan..... 204/211

Primary Examiner—John H. Mack

Assistant Examiner—Aaron Weisstuch

Attorney, Agent, or Firm—Wenderoth, Lind & Ponack

[57]

ABSTRACT

A foil of a magnetic alloy having a uniform composition is continuously manufactured by electrodepositing the desired composition as a foil on a surface of an electrically conductive endless belt in an electrodepositing bath, peeling off the resulting deposited layer and then subjecting the layer to continuous electrolytic polishing.

4 Claims, 2 Drawing Figures



PATENTED JUN 3 1975

3,887,440

*FIG. 1*



*FIG. 2*



## METHOD OF MANUFACTURING A CONTINUOUS MAGNETIC FOIL BY ELECTRODEPOSITION

### BACKGROUND OF THE INVENTION

The present invention relates to a method of manufacturing a continuous foil of magnetic material by electrodeposition.

As is well-known, the composition of an alloy deposited by electroplating, particularly in alloy plating, is greatly influenced by the current density during the electrodeposition. Therefore, in a continuous electrodeposition process, it is important to control the current density from the start to the completion of the operation in order to obtain an electrodeposited layer having a uniform alloy composition.

The above-mentioned problem is also present in the electrodeposition of Permalloy and other magnetic alloys. Particularly, in the manufacture of foils of these magnetic alloys, the magnetic characteristics of the resulting magnetic foil are greatly influenced by the alloy composition deposited, so that it is most necessary that the alloy composition of the deposited layer be uniform.

Heretofore, a magnetic alloy has been electrodeposited on a continuously moving base conductor by electrodeposition and then recovered as it is or peeled off the conductor to obtain a continuous thin film such as a foil or tape-like magnetic alloy. However, even if it is desired that the electrical or chemical conditions during the electrodeposition be constant, an abnormal current flows at points where the base conductor enters the electrodepositing bath. It is well-known that it is very difficult to prevent the occurrence of such an abnormal current.

That is, in the portion of the electrolyte where the base conductor enters the electrolyte, even if no power source is connected to the anode, a cell is partially constituted by the anode, the electrodepositing bath and the cathode, and the electrolyte surrounding the base conductor causes changes in the electrodepositing bath, whereby an abnormal current due to electrochemical reaction flows rapidly. This abnormal current is added to the normal electrodepositing current during electrodeposition. Consequently, the abnormal current acts for a certain length of time during initial electrodeposition, for example, when Permalloy is deposited to a thickness of about 2000 Å by a general electrodeposition. Therefore, there is the disadvantage that the resulting alloy composition changes in an undesirable way due to this abnormal current.

### SUMMARY OF THE INVENTION

An object of the present invention is to overcome the above described disadvantages and to improve the magnetic characteristics of magnetic foils by homogenizing the alloy composition in the direction of the thickness of a film or foil formed during continuous electrodeposition.

The inventor has recognized that in the continuous production of foils of magnetic material by electrodeposition, the portion having a non-uniform alloy composition as described above occurs mainly in the initially deposited portion of the layer, and he has made various investigations with respect to the manufacture of foils of magnetic material having a uniform alloy composition, and as a result has found that the above

described problems can be solved by providing an electrolytic polishing step subsequent to the electrodeposition stage so as to remove the initially deposited portion of the layer without technical difficulty.

Accordingly, the present invention is a method of manufacturing a continuous foil of magnetic material by electrodeposition, which comprises electrodepositing a magnetic alloy layer on a surface of an endless base conductor belt in an electrodepositing bath composed of a plurality of electrodeposition chambers, peeling off the resulting deposited layer after it has reached the desired thickness, and then subjecting the deposited layer to a continuous electrolytic polishing so as to remove the initially deposited portion thereof to leave a foil of magnetic material having a uniform composition. According to the present invention, a foil of magnetic material having a uniform alloy composition can be continuously manufactured and it is possible to improve the magnetic characteristics of the resulting foil considerably.

### BRIEF DESCRIPTION OF THE DRAWINGS

FIG. 1 is a diagrammatic view of an apparatus for practising the method of the present invention; and

FIG. 2 is a graph showing the magnetic characteristic of a foil made by the method of the present invention.

### DESCRIPTION OF THE PREFERRED EMBODIMENT

Referring to FIG. 1, an electrodepositing bath apparatus 2 comprises a plurality of electrodeposition chambers 1, 1' ... An endless base conductor belt 3 is continuously passed through the chambers 1, 1' ... of the electrodepositing bath apparatus 2. The current density in each of the electrodeposition chambers 1, 1' ... of the electrodepositing bath apparatus 2 is controlled by a current controlling device 4, whereby a magnetic alloy of the desired composition is electrodeposited on the surface of the base conductor in each electrodeposition chamber. The endless belt 3 is the base conductor for electrodeposition and can be any electrically conductive material such as stainless steel or the like. In order that the resulting deposited layer can be easily peeled off the endless belt, it is desirable that the composition of the electrodepositing bath be appropriately selected and the surface of the endless belt 3 is polished in an appropriate conventional manner to, for example, a surface roughness of less than 1  $\mu$ .

After the electrodeposition, the deposited layer is peeled off the base conductor by a peeling roller 5 or the like to obtain the layer 6. However, in this layer the alloy composition is non-uniform in the direction of the thickness thereof, as described above, and such non-uniform portion is mainly the initially deposited portion on the bottom surface of the layer 6 as seen in FIG. 1. Therefore, after removing only the initially deposited portion by means of an electrolytic polishing bath having a composition depending on the alloy composition, the composition of the remaining portion of the layer 6 is substantially homogeneous throughout.

As shown in FIG. 1, the deposited layer 6 is introduced into an electrolytic polishing bath 7 by being guided under a roller 8 so as to electrolytically polish only the initially deposited portion of the layer. After the initially deposited portion is removed in the electrolytic polishing bath 9 by a cathode 10 which is at a re-

stricted voltage, the resulting foil 11 is wound up on a winding roller in a roll 12.

The following example is given in illustration of this invention and is not intended as limitation thereof.

### EXAMPLE

Composition of electrodepositing bath based on 1 liter of water

|                         |                  |
|-------------------------|------------------|
| nickel sulfamate        | 200 cc/l.        |
| iron sulfamate          | 100 cc/l.        |
| potassium citrate       | 100 cc/l.        |
| sodium hydrogen sulfite | 3 g/l.           |
| saccharin               | 1 g/l.           |
| aqueous 28% ammonia     | regulating of pH |

Conditions of electrodeposition

|                   |                       |
|-------------------|-----------------------|
| pH                | above 9.0             |
| temperature       | above 65°C            |
| current density   | 1-5 A/dm <sup>2</sup> |
| cathodic material | stainless steel       |
| anodic material   | nickel                |

Composition of electrolytic polishing bath

|                 |                    |
|-----------------|--------------------|
| phosphoric acid | 7 parts by volume  |
| sulfuric acid   | 3 parts by volume  |
| water           | 0.8 part by volume |

Condition of electrolytic polishing

|                 |                      |
|-----------------|----------------------|
| temperature     | 80°                  |
| current density | 20 A/dm <sup>2</sup> |
| polishing time  | 10 sec.              |

A foil of magnetic material consisting of 80% Ni-20% Fe alloy and a thickness of 10 $\mu$  was obtained by using the above-described baths and under the conditions described. The thus obtained magnetic alloy had a coercive force of 2.2 Oe at 2 KHz (measuring condition 48 Oe P-P), while the coercive force prior to the electrolytic polishing of the same magnetic foil was 4.5 Oe (the measuring condition was the same as described

above).

From the B-H curve as shown in FIG. 2, it is clear that the magnetic properties of the magnetic foil obtained by the method of the present invention (curve 2) are greatly improved as compared with those of the foil produced under the same conditions, but not subjected to the electrolytic polishing treatment (curve 1).

As described above, by the method of manufacturing a continuous foil of magnetic material according to the present invention, a magnetic foil having a very uniform alloy composition can be obtained without the use of a particular base for electrodeposition and a specific electrodeposition method, so that the present invention has considerable industrial merit.

15 What is claimed is:

1. A method of manufacturing a continuous foil of magnetic material by electrodeposition, which comprises electrodepositing a desired magnetic alloy layer on a surface of an endless base conductor belt for electrodeposition in an electrodepositing bath composed of

20 a plurality of electrodeposition chambers, peeling off the resulting deposited layer in a desired thickness, and then subjecting the deposited layer to a continuous electrolytic polishing so as to remove an initially deposited portion, whereby there remains a magnetic foil of uniform composition.

2. The method as claimed in claim 1 further comprising controlling the current density in each of said electrodeposition chambers by a current controlling device.

3. The method as claimed in claim 1 wherein said belt is stainless steel.

4. The method as claimed in claim 1 wherein the surface of said belt has a roughness less than 1 $\mu$ .

\* \* \* \* \*